

May 10, 1932.

A. M. GEORGE

1,857,811

LINOLEUM AND SIMILAR HARD SURFACED FLOOR COVERING

Filed March 5, 1928



*Fig 2*



INVENTOR

Arthur M. George  
by his atty.  
Walter & Kaufman

## UNITED STATES PATENT OFFICE

ARTHUR M. GEORGE, OF LANCASTER, PENNSYLVANIA, ASSIGNOR TO ARMSTRONG CORK COMPANY, OF LANCASTER, PENNSYLVANIA, A CORPORATION OF PENNSYLVANIA

## LINOLEUM AND SIMILAR HARD SURFACED FLOOR COVERING

Application filed March 5, 1928. Serial No. 259,100.

This invention relates to flexible, hard surfaced floor covering, more particularly linoleum, and the method of making the same, inlaid linoleum being a particular example 5 of linoleum to which my invention is applicable.

In the manufacture of plain linoleum, it is customary to calender the surface with a hot roll, producing a smooth closely knit surface 10 which will resist moisture and dirt penetration. This surface may be obtained by setting the calender rolls to travel at different speeds so that a wiping action is had between the upper roll and the wearing surface, 15 whereby the top surface is ironed out smooth and closely grained. The smooth surface may also be obtained by an extrusion effect in the calender. This extrusion effect causes a relative slip between the mix and the top 20 roll whereby the wearing surface is smoothed out.

It is well recognized that moisture has a deleterious effect upon the oxidized linseed oil binder ordinarily used in the manufacture 25 of linoleum. It is also well established that alkalies and alkaline materials have an undesirable chemical reaction with the cement. Dirt which has penetrated the surface of linoleum is very difficult to remove and cannot 30 well be scraped away without injuring the surface of the goods. The hard smooth surface produced by calendering serves to obviate a good many of the defects which would attend the usage of a porous floor covering, 35 such as the penetration of undesirable chemicals, staining of the goods by liquids, and penetration of dirt.

There are certain types of linoleum, however, in which the surface is discontinuous or 40 of a porous nature. Inlaid linoleum forms a class of goods of this character, straight line inlaid linoleum forming one type, and moulded inlaid linoleum forming a different type. The straight line inlaid linoleum is formed of 45 a number of separate pieces of linoleum which are preformed to size and pressed upon a backing, the name "straight line" being derived from the clean line of juncture between adjacent pieces. Moulded inlaid linoleum is 50 formed of a granular mix applied upon a

backing where it is compressed to form a continuous web; in the moulded inlaid process, the granular mix is generally applied through stencils in order to effect a desired design and to obtain the proper depth of mix upon the 55 backing.

Straight line linoleum may be calendered and a smooth closely knit surface obtained upon the preformed pieces comprising the pattern. The lines of juncture between the 60 pieces, however, are closed by a lateral pressure which is induced by the vertical pressure of the calender or other pressure operating upon the surface of the goods to force the component pieces against the backing. 65 It will be apparent, therefore, that the full calendering pressure is not obtained upon the lines of juncture in such a direction as to force the adjacent pieces together, so the joints in inlaid linoleum are not generally as 70 strong as the intermediate parts of the cloth. The joints are likely to open if the finished linoleum is bent. This condition is particularly likely to obtain if the straight line inlaid linoleum is finished upon a flat bed press 75 instead of a calender, for the joints are less likely to be well bonded by the pressure of the press than they are by the kneading action of a calender roll.

Moulded inlaid linoleum is usually finished 80 under a flat press so the granular mix is compressed into a continuous web, while the design in different shades or colors is retained, since the flat bed press will not smear adjacent colors to any great extent, nor will 85 it distort geometrical designs made of pul- verulent material as a calender roll might do.

Because of this difference in the manufacturing process, and the differences in the form of 90 material used to make the product, moulded inlaid material is somewhat more porous than calendered linoleum. It does not get the benefit of the kneading extruding action of a calender roll, nor does it get a slipping, ironing effect of such a roll on its wearing 95 surface. Moreover, if the moulded inlaid material be embossed, a calendered surface cannot be had, for the surface is irregular.

It will thus be seen that inlaid linoleum 100 is more likely to be subject to staining and

infiltration of moisture and undesired chemical agents than is ordinary plain linoleum. The susceptibility of inlaid linoleum to these undesired effects may be due to the porous nature of moulded material or to crack lines formed at the line of juncture of the pieces comprising straight line inlaid linoleum.

I obviate the foregoing defects by the application of a coating of water and alkali resistant material which fills the surface pores of moulded linoleum and closes any cracks which may occur at the line of juncture in straight line inlaid goods. The coating is preferably alkali resistant as applied to linoleum formed with an oxidized linseed oil binder, since alkaline materials tend to break down such a material and destroy the linoleum. The coating should be sufficiently fluid that it will penetrate the pores of the material and form an effective seal against any subsequent liquid infiltration. Moreover, the coating should be sufficiently hard that dirt will not be ground into the surface of the goods in ordinary usage.

In the accompanying drawings illustrating a preferred method and apparatus for carrying out my invention;

Figure 1 shows a side elevation partly broken away of a machine for applying a coating according to my invention; the figure being more or less diagrammatic; and

Figure 2 is a top plan view of a portion of Figure 1, the exhaust hood being removed.

Referring to the illustrated embodiment, there is shown a strip 2 of linoleum which passes from a roll 3 across guide rollers 4 and 5 to a travelling conveyor 6. Between the guide rollers 5 and the conveyor 6 there is interposed a pair of rolls 7 and 8 which are connected together, as indicated diagrammatically, by chain line 9. The top roll 7 is adjustable vertically with respect to the lower roll 8 by means of a suitable screw adjustment 10, whereby various gauges of material may be accommodated and various degrees of coating may be applied to the linoleum by the top roll 7.

The top roll 7 is preferably formed with an outer covering 11 of rubber or similar material of a resilient nature so that when linoleum is introduced between the rolls 7 and 8, the resiliency of the roll 7 will compensate for any unevenness in the surface of the linoleum. It will be understood that the face or the wearing surface of the linoleum is on top as viewed in the figures illustrating the invention.

At each end of the top roll 7, but inside the edges of the linoleum 2, I place guards 12 which conform to the curvature of the roll 7 and ride on top of the linoleum 2. The coating material is placed on the linoleum 2 immediately in front of the resilient roll 7 and between the guards 12 and lies there as a pool from which a small amount is

drawn continuously as the roll 7 revolves in contact with the cloth going to the right as shown in the drawings.

The rolls 7 and 8 are driven by a suitable power source 13 which also serves to drive the conveyor 6, so that the speed of the conveyor 6 is correct to receive cloth coming from the rolls 7 and 8 and draw the cloth from the rolls without buckling. That is to say, I prefer that the conveyor 6 travel slightly faster than the speed of the goods discharged from the coating roll 7.

I find that the linoleum passing between the coating roll 7 and the backing roll 8 travels at a speed more nearly that of the backing roll 8 than the coating roll 7, if these rolls are traveling at a different speed. It seems that the coating acts as a lubricant which causes the roll 7 to slip, thereby giving a thinner coating to the face of the linoleum. I prefer to drive the coating roll at a speed slightly less than the speed of the backing roll 8 so that a wiping action will be obtained between the coating roll 7 and the face of the goods. This serves to remove any excess of coating material and gives a well coated piece of goods without too much coating material appearing on the face of the goods to materially alter the natural finish of the face.

The backing roll 8 is preferably made of some rigid material such as steel in order that irregularities in the thickness of the cloth may be compensated for by the resilience of the coating roll 7. This insures that an irregularity in thickness of material will not cause noticeable irregularity in the thickness of the coating.

In order to harden the coating as quickly as possible, in order to facilitate handling of the coated linoleum, I provide a hood 14 which extends substantially the length of the conveyor 6. This hood is provided with a plurality of ducts 15 which serve to draw air from the surface of the coated linoleum; an exhaust fan 16 being used to withdraw the air. Intermediate the ducts, I provide inlet passages 17 for air which will be swept across the face of the coated linoleum. Within these inlet passages, I place suitable heating coils 18, such as steam coils, in order to facilitate evaporation of the solvent in the coating.

In coating different types of linoleum, I prefer to use different types of coating rollers 7, correcting the hardness of the resilient coating 11 of the roll 7 to the type of linoleum to be coated. The hardness of the roll 7 will of course be dependent upon the fluidity of the coating material and upon the irregularity or smoothness of the face to be coated. In coating an embossed piece of linoleum having depressions in the surface, I use a relatively soft coating roll. In coat-

ing a relatively smooth piece of plain linoleum, however, I prefer a harder roll.

In manufacturing my improved linoleum, I prefer to form the inlaid goods in the usual way, maturing them to obtain a hard surface and then apply a coating having the desired characteristics.

I prefer to use a quick drying lacquer which will penetrate the pores in the moulded material and fill up any cracks in straight line goods. By using a quick drying lacquer, the filling operation may be quickly and conveniently carried out, the interstices being filled and the coating dried as a continuous operation while the floor covering is moving along a traveling carrying belt.

A lacquer which I have found to give satisfactory results can be made according to the following formula using one-half second

20 cotton:

|                        | Parts |
|------------------------|-------|
| Nitrated cotton        | 10    |
| Ester gum              | 10    |
| 25 Tricresyl phosphate | 1     |
| Castor oil             | 4     |
| Ethyl acetate          | 25    |
| Absolute alcohol       | 50    |

The above proportions are by weight.

30 I have found that numerous changes may be made in the above formula without materially changing the characteristics of the finished linoleum, for example, 10 parts of absolute alcohol might be substituted with 10 parts butanol.

A quick drying adhesive coating which penetrates the cracks in the straight line goods is advantageous in that the lines of juncture between the pieces comprising the material 40 will be effectively closed prior to the rolling of the goods for shipment. Straight line inlaid linoleum is liable to open at the seams at the joints between the surface portions if the goods be bent, the flexibility of the material being sufficient to prevent cracking intermediate the joints. In my improved straight line inlaid linoleum, the joints do not open so readily and a substantially continuous surface is obtained irrespective of the 50 bending or other manipulation of the cloth.

A film of the coating may be left on the surface of the floor covering if desired. I prefer, however, to apply a relatively thin coating so that the surface texture is not materially altered; the dull natural surface of linoleum is more ornamental than the glossy bright, shiny surface of varnishes or lacquer, particularly in the case of embossed inlays such as described in Patent #1,630,085, of 60 May 24, 1927. The coating varnish or lacquer, should be quite fluid so that it will penetrate the interstices of the linoleum, binding the component portions of the goods together at the surface, thereby preventing the infiltration of undesired materials. The fluidity

of the coating also determines to some extent the thickness of the film left on the surface of the goods. The film remaining on the surface of the goods should be relatively thin so that it will not materially alter the coloring of 70 the pattern, or change the surface texture of the goods.

It is desirable that the coating be transparent in thin layers so that any of the coating which may overlie the linoleum will not 75 change the color of the pattern to any great extent. Shadings of colors may be obtained if desired by tinting or dyeing the coating; but the coating is primarily a sealing agent.

Although coatings other than lacquer may be used to fill the pores of the linoleum, I prefer nitrocellulose lacquer because of its quick drying properties; its ready availability; and its susceptibility to the use of solvents such as appearing in formula above 85 which have a solution effect on the linoleum binder. This solution effect enhances the effect of the coating inasmuch as it augments the degree of penetration which would be obtained by mere mechanical methods of application. The total wear of the coating and the linoleum is increased by mutual contribution of each to the other since the coating penetrates below the surface and there is a more or less interlaced structure. Moreover, 90 the unsightliness of lanes of traffic is reduced and the repair of such areas is made easier and more satisfactory because the more penetrating material is absorbed to an imperceptible degree from the surface inward, 95 hence it is never completely worn off in conspicuous spots as would be the case with a purely superficial coating. These advantages are attributable to some measure to the solvent action on the linoleum cement of 100 those solvents used for nitrocellulose lacquer as distinguished from turpentine and petroleum distillates used in varnishes; the latter have considerable less solvent action and are not quite so desirable from a penetration 105 standpoint.

Various types of lacquers may be employed and the newer solvents such as the benzene hydrocarbons (e. g. benzol, toluol, xylol); the alcohols (e. g. methyl, ethyl, butyl); the esters (e. g. methyl-, ethyl-, butyl-acetates, or butyrates); the ketones (e. g. acetone, methyl-ethyl ketone); the ethers (e. g. ethyl ether and glycol ethers) and similar solvents are much more penetrating and give 115 results on linoleum not obtainable with the varnish solvents, and a degree of penetration far in excess of that obtained with the same materials on less porous surface such as paints and enamels.

120 After the solvent has evaporated, the solid matter remaining may be any of the esters or ethers of cellulose, oils, oleo-resins or synthetic resins. The use of plasticizers will of course depend upon the nature of the solid 125

matter selected. It will be apparent that the degree of penetration depends upon the proper choice of solvents rather than upon the exact nature of the dissolved body matter.

5 The sealing coat should be flexible so that it will not break away from the floor covering when the linoleum is bent. The effect of a coating of this character, which bonds with the material comprising the floor covering 10 is to close the seams between adjacent portions in the straight line inlaid linoleum and to strengthen those sections which are partly closed. In any event the coating forms a sealing agent which effectively stops the 15 pores and seam openings which may be present. By using a coating which adheres firmly to the material of the floor covering and which is flexible, I completely seal the seams and pores of the floor covering against moisture, destructive chemical agents and dirt 20 which might penetrate the wearing surface. Moreover, the linoleum is less liable to staining or discoloration. The surface is easier 25 to keep clean since those particles of dirt which lie upon it cannot penetrate into the pores or other openings in the goods.

The sealing coating is beneficial as applied 30 to all types of linoleum floor covering preserving the interior from moisture and chemical attack. Inlaid linoleum including an oxidized linseed oil binder is perhaps the best example of the utility of my invention, for such a covering is subject to frequent 35 washings and to various soaps which are harmful to the binder.

I am aware that it has been customary to 40 wax linoleum, but my improved coating is to be distinguished from wax or varnish as may have been hitherto used, in that waxes and varnishes having a turpentine solvent 45 have little or no penetrating power since they have a relatively low "wetting power" or relatively high surface tension, and the solvent action on the linoleum ingredients is practically negligible.

The thin layer of the coating which may 50 overlie the treated surface may be ground off or left to wear off. If the overlying surface is left to wear off, the worn places may be made to match the unworn places by waxing 55 or by the application of additional coating material. A complete layer of the coating will of course protect the entire surface and those portions intermediate the pores, from moisture, alkali and stains and is desirable from that standpoint.

While I have illustrated and described the 60 present preferred embodiment of my invention, it will be understood that the invention is not limited thereto, but may be otherwise practiced and embodied within the scope of the following claims.

I claim:

65 1. The method of making a stain and moisture resistant linoleum, comprising compress-

ing individual quantities of floor covering mix to form a continuous web, and sealing the openings in the surface of the web with a dissolved sealing material the solvent of which has a dissolving action on the web 70 whereby the sealing material is bonded with the web and penetrates the openings of the web.

2. The method of making a stain and moisture resistant moulded inlaid linoleum comprising, compressing granulated linoleum mix to form a substantially continuous web, maturing the web so formed, forcing a dissolved sealing material against the surface of the web, the solvent of the sealing material having a dissolving action on the linoleum binder, removing the excess sealing material from the web, and evaporating the solvent whereby the moulded inlaid linoleum is formed with its surface pores sealed with plugs which 85 are bonded with the linoleum.

3. In the method of making a flexible hard surfaced floor covering, the steps consisting in forming a body of a filler and a binder by compression, and applying a coating containing a solvent having a dissolving action on the binder.

4. In the method of making a flexible hard surfaced floor covering, the steps consisting in forming a body sheet from a filler and a linseed oil binder, maturing the body sheet to harden the linseed oil binder, and applying a nitrocellulose lacquer coating in a solvent having a solvent action on the matured 100 binder.

5. As a new article of manufacture, a hard pressed web comprising a hardened linseed oil binder and fillers, said web having surface pores therein, and an alkali resistant coating substantially sealing all of said pores, 105 said coating being bonded to the web by a mixture of the coating and the binder.

In witness whereof I have hereunto set my hand.

ARTHUR M. GEORGE. 110

115

120

125

130